# EUROPEAN PATENT SPECIFICATION

(11) **EP 0 325 610 B1**
(45) Date of publication and mention of the grant of the patent: **06.04.1994**
(21) Application number: 87906715.5
(22) Date of filing: 25.09.1987
(51) Int. Cl.: D06M 13/244, D06M 13/282, D06M 13/432, D06M 15/43

(54) **FLAME-RESISTANT COTTON BLEND FABRICS**
FLAMMWIDRIGE BAUMWOLLMISCHGEWEBE
TISSUS EN COTON MELANGE RESISTANT AUX FLAMMES

(30) Priority: 26.09.1986 US 911720; 28.10.1986 US 923965
(43) Date of publication of application: 02.08.1989
(73) Proprietor: Burlington Industries, Inc., Greensboro North Carolina 27420 (US)
(72) Inventor: HAUSER, Peter, J., Greensboro, NC 27410 (US); TRIPLETT, Benny, L., Pleasant Garden, NC 27313 (US); SUJARIT, Chumpon, High Point, NC 27260 (US); HANSEN, John, H., Greensboro, NC 20410 (US); JOHNSON, James, R., McLeansville, NC 27310 (US)
(74) Representative: Sturt, Clifford Mark
(86) International application number: US8702432
(87) International publication number: WO8802283

(56) References cited:
- US-A- 3 897 584
- US-A- 3 974 310
- US-A- 4 166 897
- US-A- 4 448 817
- US-A- 4 494 951
- AMERICAN DYESTUFF REPORTER, vol. 65, no. 21, January 1976, pages 33,34,63; S.L.VAIL et al.: "Topping of THPOH-NH3 fire-retardant finishes"
- THE JOURNAL OF FIRE RETARDANT CHEMISTRY, vol. 6, August 1979, pages 149-166,Wesport, US; R.H. BARKER et al.: "Calorimetric study of polyester/cotton blend fabrics. III. Effects of binary retardant systems"

## Description

This invention relates to a process for imparting flame-retardant properties to cotton/synthetic fiber blends, specifically polyester/cotton fabrics, using two flame-retardant chemicals or flame-retardant systems, one specific to the synthetic component and the other specific to the cotton component.

### BACKGROUND OF THE INVENTION

Prior attempts to achieve acceptable flame-resistant polyester/cotton or nylon/cotton blends have not met with commercial success. None of the treatments is practical from the consumer point of view, producing fabrics that have a very stiff hand. This is because in order to achieve the requisite flame-resistant properties, a high chemical add-on is required. This add-on makes the fabric stiff, masks the color of the underlying fabric, and often imparts an acrid or unacceptable odor to the fabric. In addition, the performance of the flame-resistant fabrics is often unreliable.

Most of the previous work conducted on flame-resistant polyester/cotton or nylon/cotton blends used a single chemical system that was targeted for the cotton component of the blend. The approach was to "load" the fabrics with a flame retardant specific for cotton, for instance THPS [tetrakis-(hydroxymethyl)phosphonium sulfate]. It was not unusual with these earlier products to use from 30 to 35% of fixed chemical add-on in order for the polyester/cotton or nylon/cotton blend fabric to pass a bottom vertical flame test. Regrettably, however, the aesthetics of the finished fabrics were poor, as they has a very stiff hand and the appearance of a coated fabric. The add-ons used for these products were far in excess of the theoretically required amounts.

When THPS is applied to a polyester/cotton or nylon/cotton blend, a degree of flame resistance results, but it remains stiff and generally unacceptable. Since the THPS is specific to cotton, it does not react with the polyester or nylon content of the fabric but simply physically coats the synthetic component. As a result, after multiple launderings, that portion of the flame retardant surrounding the polyester or nylon fiber is partially lost. In consequence, it was not unusual to use as much as 5.5% phosphorus add-on for a polyester/cotton blend, at least initially, in order to result in the target 3% of fixed phosphorus after 50 launderings in hot water.

In the 1970's, polyester/cotton blends were flame retarded using tris-2,3-dibromopropyl phosphate ("Tris") in combination with THPS. However, "Tris" was found to be a carcinogen and was withdrawn from the market, so that there is no predominantly-polyester blend of polyester and cotton sold today that has been treated with flame-retardant chemicals. An object of the present invention is to produce acceptable flame-resistant polyester/cotton blends using multiple flame-retardant chemicals or chemical systems, and to employ processing conditions or adjuvants that produce a commercially acceptable, attractive product having good color and acceptable hand.

### BRIEF DESCRIPTION OF THE INVENTION

The process of the present invention employs two flame-retardant (FR) systems, one specific to the synthetic component and the other specific to the cotton component of the synthetic/cotton blends being flame-retarded. With this approach, the amount of flame retardant, such as THPS, required to satisfy flame-resistance standards can be reduced significantly and the resulting fabrics have not only better flame resistance, but also better aesthetics. In the processes disclosed in more detail below, different flame-retardant chemicals are applied in separate processing steps. Processing conditions, especially temperatures and humidities, are carefully controlled in order to optimize the use of the flame-retardant chemicals and to ensure good fixation to the synthetic/cotton blends, even after several launderings.

The polyester/cotton blends treated in accordance with the present invention contain between 35% and 80% of polyester, the balance being cotton.

The term "polyester" is used in its usual sense to mean highly polymeric, essentially linear polyester resins made by the reaction of a dicarboxylic acid or ester with a diol in the presence of an esterification or ester interchange catalyst. Illustrative dicarboxylic acids are malonic, succinic, adipic, azelaic, maleic, fumaric, hydromuconic, isophthalic, terephthalic, and cyclohexane-dicarboxylic acids. Representative diols are ethylene glycol, propylene glycol, butylene glycol and 1,6-hexanediol. See US-A-2,465,319 and US-A-2,901,446. The common commercial polyester resins are polyethylene terephthalate and polyethylene terephthalate modified by inclusion of minor proportions of a different glycol or dicarboxylic acid during the polyesterification process. The polyester used in the working examples that follow was polyethylene terephthalate.

As used in this specification, the term "nylon" is used to describe a manufactured fiber in which the fiber-forming substances are long-chain synthetic polyamides having recurring polyamide groups (-CONH-) as an integral part of the polymer chain. These polyamides are formed from various combinations of diacids, diamines and amino acids. See generally Kirk-Othmer Encyclopedia of Chemical Technology, Vol. 16 (Interscience, New York, 2nd. ed., 1968) pp. 1-105.

The polyester/cotton fibrous materials which can be provided with a flame-retardant finish according to the invention can be in any desired stage of processing, i.e., they can be treated as woven or knitted fabrics, dyed or undyed, or as textiles which have already been further processed.

Flame-resistant properties are imparted to the fabric in two distinct steps, one for the cotton component and the other for the polyester component. The specific procedures of the process of the invention are now described.

### I. Treating the Cotton Component of the Synthetic/Cotton Blend

Flame-resistant properties are imparted to the cotton component of the synthetic/cotton blend by impregnating the fabric with an aqueous solution containing a pre-condensate of a carefully measured quantity of urea [NH₂COHN₂] and a tetrakis(hydroxymethyl) phosphonium salt, referred to as THP, as THPS when the salt is the sulphate [(HOCH₂)₄P⁺]₂SO₄⁼ or THPC when the salt is the chloride; the oxalate and phosphate salts are also known. The THP salt/urea precondensate is applied to the fabric and dried to a specific moisture level. It is then reacted on the fabric with ammonia, usually ammonia gas, under controlled conditions to form an ammoniated flame retardant which, in turn, is oxidised, usually with hydrogen peroxide, to form a three-dimensional flame retardant polymer network within the cotton fibre structure. This process results in a fabric having a softer hand than other treatments, such as THPS/urea, which tends to stay on the outside of the fibres and stiffen the fibres and is more susceptible to removal by repeated laundering.

Currently there are two THP-based flame retardant systems marketed for this type of treatment. **Pyroset** (Registered Trade Mark) TPO is a THPS/urea precondensate of tetrakis-(hydroxymethyl) phosphonium sulphate and urea available from American Cyanamid Co., while **Retardol AC** (Registered Trade Mark) is a THPC/urea prepolymer condensate of tetrakis-(hydroxymethyl) phosphonium chloride and urea available from Albright & Wilson.

The process of imparting flame resistance to 100% cotton fabrics using THPS/urea (Retardol AC) is known as the **PROBAN** porches as licenced by Albright & Wilson. The THP salt/urea precondensate process itself is described in the following US patents: 4,078,101; 4,145,463; 4,311,855 and 4,494,951, all to Albright & Wilson. This process is considered effective and is widely promoted by at least two US companies for imparting flame resistance to 100% cotton fabrics. The THP salt/urea precondensate process by itself is ineffective to adequately protect polyester/cotton blends containing more than about 35 to 40% polyester as discussed previously.

### II. Flame Retardant Treatments for Polyester

One of the following flame retardants may be used for the polyester component of the blend. Hexabromocyclododecane is available as CD-75 from Great Lakes Chemical and as Saytex HBCD from the Ethyl Corporation. It is sold primarily for use as a flame retardant for plastics, in part because of its poor solubility in solvents commonly used for textile processing. Hexabromocyclododecane melts at about 182°C (360° F), and, when applied as a dispersion to a polyester/cotton fabric at elevated temperatures above its melting point, then cooled, hexabromocyclododecane fuses to the fiber, imparting the requisite flame-resistant properties to the fibers of the polyester.

Another flame retardant material used in accordance with the present invention specific for the polyester component of the fabric is a thermally stable cyclic phosphonate ester prepared by reacting alkyl-halogen-free esters with a bicyclic phosphite. As a class, these cyclic phosphonate esters are represented by one of the formulas:
where a is 0 or 1; b is 0, 1 or 2, c is 1, 2 or 3 and $\text{a+b+c}$ is 3; R and R' are the same or different and are alkyl (C₁-C₈), phenyl, halophenyl, hydroxyphenyl, tolyl, xylyl, benzyl, phenethyl, hydroxyethyl, phenoxyethyl, or dibromophenoxymethyl; R₂ is alkyl (C₁-C₄); and R³ is lower alkyl (C₁-C₄) or hydroxyalkyl (C₁-C₄) or
where d is 0, 1 or 2; e is 1, 2 or 3; R² is alkyl (C₁-C₄); R³ is lower alkyl (C₁-C₄) or hydroxyalkyl (C₁-C₄); R⁴ is alkyl (C₁-C₄) phenyl, halophenyl, hydroxyphenyl, hydroxyethyl, phenoxyethyl, dibromophenoxymethyl, tolyl, xylyl, benzyl or phenethyl; and R⁵ is monovalent alkyl (C₁-C₆), chlorophenyl, bromophenyl, dibromophenyl, tribromophenyl, hydroxyphenyl, naphthyl, tolyl, xylyl, benzyl, or phenethyl; divalent alkylene (C₁-C₆), vinylene, o-phenylene, m-phenylene, p-phenylene, tetrachlorophenylene (o, m, p), or tetrabromophenylene (o, m, or p); or trivalent phenyl.

The preferred compounds are represented by the formula:
in which X is 0 or 1, and usually a 50:50 mixture of the mono- and di-esters. The preparation of these cyclic phosphonate esters and their use as flame retardants are described in US-A-3,789,091 and US-A-3,849,368, the disclosures of which are hereby incorporated by reference.

**Antiblaze 19T**, as described by the supplier Albright & Wilson Inc., of Richmond, Virginia, U.S.A., is a cyclic phosphonate ester, available as an odorless viscous liquid (viscosity 250 PA.s) with a flashpoint of 171°C (340°F) (ASTM D-93).

**Hexabromocyclododecane**, as described by its supplier Great Lakes Chemical Corporation of West Lafayette, Indiana, U.S.A., is a cyclic alkyl bromide, empirical formula C₁₂H₁₈Br₆, CAS registry number 25637-99-4, composed of hexabromocyclododecane and related bromocycloalkanes. It is an odorless, Water-insoluble, off-white powder having a melting point range of 142-182°C (288-360°F) and is preferably used in the process of this invention as a dispersion in water or an aqueous pad bath system.

Tetrakis-(hydroxymethyl)phosphonium chloride/urea prepolymer condensate (**THPC/urea**) is available from Albright & Wilson, Inc., under the name **Retardol AC**. A related chemical, THPS/urea prepolymer condensate, is available from American Cyanamid Co., under the name of **Pyroset TPO**.

**Aerotex H** is described by its supplier, American Cyanamid Co., as a cationic product with nonionic and anionic moieties, and is included in the pad bath formulation as a softener.

**TMN-10** is ethoxylated 2,6,8-trimethylnonanol, commercially available from Union Carbide Corporation.

### Flame Resistance Testing Methods -- the following testing procedure was used:

**FR Federal Test Method 5903** is intended for use in determining the resistance of cloth to flame and glow propagation and tendency to char. A rectangular cloth test specimen (70mm x 120mm) with the long dimension parallel to the warp or fill direction is placed in a holder and suspended vertically in a cabinet with the lower end 1.9 cm above the top of a Fisher gas burner. A synthetic gas mixture consisting primarily of hydrogen and methane is supplied to the burner. After the specimen is mounted in the cabinet and the door closed, the burner flame is applied vertically at the middle of the lower edge of the specimen for 12 seconds. The specimen continues to flame after the burner is extinguished. The time in seconds the specimen continues to glow after the specimen has ceased to flame is reported as afterglow time; if the specimen glows for more than 30 seconds, it is removed from the test cabinet, taking care not to fan the glow, and suspended in a draft-free area in the same vertical position as in the test cabinet. Char length, the distance (in centimeters) from the end of the specimen, which was exposed to the flame, to the end of a lengthwise tear through the center of the charred area to the highest peak in the charred area, is also measured. Five specimens from each sample are usually measured and the results averaged.

As used throughout this specification and the claims that follow, all parts and percentages are expressed by weight and all temperatures reported in degrees C, unless otherwise indicated. The invention will be furhter illustrated with reference to the following examples:

### Comparative Example 1A

Fabric style 9886 (50/50 nylon/cotton) was padded to a wet pickup of 61% with Pyroset TPO (THPS-urea precondensate from American Cyanamid; see bath formula), and heated at 54°C for 48 seconds. The moisture content was found to be 15.5-16% as measured with a Mahlo meter. The fabric was equilibrated in a plastic bag for 1-2 hours. The fabric was then exposed to ammonia gas at 6:1 ammonia: phosphorus mole ratio. Oxidation of the fabric by a hydrogen peroxide/sodium silicate solution followed. The amount of peroxide used was 5% on the weight of fabric. The sodium silicate was used to maintain a pH of 9-9.5. The fabric was rinsed and tumble dried.

| Bath formula: | |
|---|---|
| Water | 30.6% |
| Aerosol C 61 wetting agent | 0.2% |
| Sodium acetate (60%) | 0.5% |
| Pyroset TPO | 68.7% |

The TPO/ammonia-treated style 9886 fabric was subsequently padded with a 15% Antiblaze 19 (Albright & Wilson) solution, heated in an oven at 193°C for 45 seconds and tested for flame resistance as prepared and after 25 launderings.

| Fabric | FTM 5903 | (Char Length) |
|---|---|---|
| | O Laund. | 25 Laund. |
| 9886+TPO/ammonia+AB19 | 5 cm | 11.4 cm |

### Comparative Example 1B

The TP0/ammonia-treated style 9886 fabric of comparative Example 1A was also subsequently padded with a 15% dispersion of hexabromocyclododecane (HBCD), heated at 182°C (360°F) for 45 seconds, and tested for flame resistance as prepared and after 25 launderings.

| Fabric | FTM 5903 | (Char Length) |
|---|---|---|
| | O Laund. | 25 Laund. |
| 9886+TPO/ammonia+HBCD | 7 cm. | 7-7.6 cm. |

None of the treated fabrics of comparative Example 1A or 1B exhibited either afterflame or afterglow. The results show a high level of flame resistance, and the treated fabrics had satisfactory aesthetic properties.

### Example 1

In experiments similar to comparative Example 1, 65/35 polyester/cotton fabric, style 9798, and 40/60 polyester/cotton fabric, style 9496, were padded with Pyroset TPO; see bath formula. The fabrics were dried to 16-16.5% moisture content, as measured with a Mahlo meter. The fabrics were then exposed to ammonia gas at a >6:1 ammonia:phosphorus mole ratio. Oxidation of the fabric by a hydrogen peroxide/sodium silicate solution followed. The amount of peroxide used was 5% on the weight of fabric. The sodium silicate was used to maintain a pH of 9-9.5. The fabric was rinsed and tumble dried.

| Bath Formula: | |
|---|---|
| Water | 52.5% |
| Aerosol C 61 wetting agent | 0.2% |
| Aerotex H softener | 2.0% |
| Sodium acetate | 0.3% |
| Pyroset TPO | 45.0% |

| Fabric | Wet Pickup |
|---|---|
| 9798 | 61% |
| 9496 | 63% |

Both TPO/ammonia-treated fabrics were subsequently padded with a 15% dispersion of hexabromocyclododecane (HBCD), heated at 182°C (360°F) for 45 seconds, and tested for flame resistance as prepared and after 25 launderings.

| Fabric | FTM 5903 | (Char Length) |
|---|---|---|
| | O Laund. | 25 Laund. |
| 9798+TPO/ammonia+HBCD | 6.3 cm. | 5.6 cm. |
| 9494+TPO/ammonia+HBCD | 5.0 cm. | 5.0 cm. |

None of the samples tested exhibited either afterflame or afterglow, and the low char lengths indicate a high level of flame resistance. The treated fabrics had a satisfactory hand and appearance.

## Claims

1. A process for imparting wash-fast flame-resistance to a polyester/cotton blend fabric that remains after multiple launderings, comprising:
applying (a) a first flame retardant consisting of a prepolymer condensate of urea and a tetrakis-(hydroxymethyl) phosphonium salt for imparting flame resistance to the cotton fibres, exposing the prepolymer condensate-containing fabric to a source of ammonia to form an ammoniated prepolymer, then oxidising the ammoniated prepolymer to form a flame-retardant polymer network within the cotton fibre structure; followed by applying (b) a second flame retardant consisting of (1) a cyclic phosphonate ester or (2) hexabromocyclododecane for imparting flame resistance to the polyester fibres; and
curing the fabric at elevated temperatures thereby fixing the applied cyclic phosphonate ester or hexabromocyclododecane to the polyester fibres.

2. A process as claimed in claim 1, in which the tetrakis-(hydroxymethyl) phosphonium salt is the chloride salt.

3. A process as claimed in claim 1, in which the tetrakis-(hydroxymethyl) phosphonium salt is the sulphate salt.

4. A process as claimed in claim 1, in which the tetrakis-(hydroxymethyl) phosphonium salt is the oxalate salt.

5. A process as claimed in claim 1, in which the tetrakis-(hydroxymethyl) phosphonium salt is the phosphate salt.

6. A process as claimed in any one of the preceding claims, in which the cyclic phosphonate ester is represented by the formula: in which X is 0 or 1.

7. A process as claimed in any one of claims 1 to 5, in which the flame retardant in step (b) is hexabromocyclododecane.

8. A process as claimed in claim 7, in which the hexabromocyclododecane is applied as an aqueous dispersion and is cured at a temperature of at least about 182°C (360°F) to melt and fuse the hexabromocyclododecane to the polyester or nylon fibres.

9. A process as claimed in any one of claims 1 to 8, in which the blend contains from about 35% to about 80% polyester, balance substantially entirely cotton.

## Patentansprüche

1. Verfahren, um einem Polyester/Baumwollmischgewebe waschechte, flammhemmende Eigenschaft zu verleihen, die viele Wäschen überdauert, das umfaßt:
Auftragen (a) eines ersten flammhemmenden Mittels, das aus einem Vorpolymerisatkondensat aus Urea und einem Tetrakis-(Hydroxymethyl) Phosphoniumsalz besteht, um den Baumwollfasern flammhemmende Eigenschaft zu verleihen, Aussetzen des Vorpolymerisatkondensat-enthaltenden Gewebes gegenüber einer Ammoniakquelle, um ein ammoniakhaltiges Vorpolymerisat auszubilden, danach Oxidieren des ammoniakhaltigen Vorpolymerisats, um ein flammhemmendes Polymer-Netzwerk innerhalb der Baumwollfaserstruktur auszubilden; gefolgt durch ein Auftragen (b) eines zweiten flammhemmenden Mittels, das aus (1) einem zyklischen Phosphonat-Ester oder (2) Hexabromocyclododekan besteht, um den Polyesterfasern flammhemmende Eigenschaft zu verleihen; und
Imprägnieren (curing) des Gewebes bei erhöhten Temperaturen, wodurch das aufgetragene zyklische Phosphonat-Ester oder Hexabromocyclododekan an den Polyesterfasern fixiert wird.

2. Verfahren gemäß Anspruch 1, worin das Tetrakis-(Hydroxymethyl) Phosphoniumsalz das Chloridsalz ist.

3. Verfahren gemäß Anspruch 1, worin das Tetrakis-(Hydroxymethyl) Phosphoniumsalz das Sulfatsalz ist.

4. Verfahren gemäß Anspruch 1, worin das Tetrakis-(Hydroxymethyl) Phosphoniumsalz das Oxalatsalz ist.

5. Verfahren gemäß Anspruch 1, worin das Tetrakis-(Hydroxymethyl) Phosphoniumsalz das Phosphatsalz ist.

6. Verfahren gemäß einem der vorhergehenden Ansprüche, worin das zyklische Phosphonat Ester durch die Formel dargestellt wird: in der X 0 oder 1 ist.

7. Verfahren gemäß einem der Ansprüche 1 bis 5, worin das flammhemmende Mittel in Verfahrensschritt (b) Hexobromocyclododekan ist.

8. Verfahren gemäß Anspruch 7, worin das Hexabromocyclododekan als eine wässrige Dispersion angewandt wird und bei einer Temperatur von mindestens ca. 182° C (360° F) imprägniert wird, um das Hexabromocyclododekan zu schmelzen und an die Polyester- oder Nylonfasern einzuschmelzen.

9. Verfahren gemäß einem der Ansprüche 1 bis 8, worin das Gemisch von ca. 35 % bis ca. 80 % Polyester enthält und die Differenz im wesentlichen ganz aus Baumwolle besteht.

## Revendications

1. Procédé pour conférer des propriétés de résistance à la flamme et de solidité au lavage à un tissu mélangé de polyester et de coton, ces propriétés se conservant après plusieurs blanchissages, qui consiste :
à appliquer (a) un premier retardateur de flamme, constitué d'un condensat prépolymère de l'urée et d'un sel de tétrakis-(hydroxyméthyl)phosphonium, pour conférer aux fibres de coton des propriétés de résistance à la flamme, à exposer le tissu, contenant le condensat prépolymère, à une source d'ammoniac pour former un prépolymère ammonié, puis à oxyder le prépolymère ammonié pour former un réseau polymère retardateur de flamme à l'intérieur de la structure des fibres de coton ; puis à appliquer (b) un deuxième retardateur de flamme constitué (1) d'un ester phosphonate cyclique ou (2) d'hexabromocyclododécane, pour conférer aux fibres de polyester une propriété de résistance à la flamme , et
à traiter le tissu à haute température, pour fixer sur les fibres de polyester l'ester phosphonate cyclique ou l'hexabromocyclododécane déjà appliqué.

2. Procédé selon la revendication 1, dans lequel le sel de tétrakis-(hydroxyméthyl)phosphonium est le chlorure.

3. Procédé selon la revendication 1, dans lequel le sel de tétrakis-(hydroxyméthyl)phosphonium est le sulfate.

4. Procédé selon la revendication 1, dans lequel le sel de tétrakis-(hydroxyméthyl)phosphonium est l'oxalate.

5. Procédé selon la revendication 1, dans lequel le sel de tétrakis-(hydroxyméthyl)phosphonium est le phosphate.

6. Procédé selon l'une quelconque des revendications précédentes, dans lequel l'ester phosphonate cyclique est représenté par la formule suivante : dans, laquelle X vaut 0 ou 1.

7. Procédé selon l'une quelconque des revendications 1 à 5, dans lequel le retardateur de flamme l'étape (b) est l'hèxabromocyclododécane.

8. Procédé selon la revendication 7, dans lequel l'hexabromocyclododécane est appliqué en dispersion aqueuse et est traité à une température d'au moins environ 182°C (360°F), pour subir une fusion et fusionner l'hexabromocyclododécane aux fibres de polyester ou de nylon.

9. Procédé selon l'une quelconque des revendications 1 à 8, dans lequel le mélange contient d'environ 35 % à environ 80 % de polyester, le reste étant, dans sa grande totalité, constitué de coton.
